

A. ROBINSON.  
PREPARATION OF ROOFING FABRIC.  
No. 48,311.

Patented June 20, 1865.

Fig: 2.



Fig: 1.



Witnesses:

Geo. Harold

Chas. C. Smith

Inventor:  
Alfred Robinson

# UNITED STATES PATENT OFFICE.

ALFRED ROBINSON, OF NEW YORK, N. Y.

## IMPROVED MODE OF PREPARING ROOFING MATERIAL.

Specification forming part of Letters Patent No. 48,311, dated June 20, 1865.

*To all whom it may concern:*

Be it known that I, ALFRED ROBINSON, of the city and State of New York, have invented, made, and applied to use a certain new and useful Improvement in Preparing Roofing Fabrics; and I do hereby declare the following to be a full, clear, and exact description of the said invention, reference being had to the annexed drawings, making part of this specification, wherein—

Figure 1 is a plan of the machine employed by me, and Fig. 2 is a vertical longitudinal section of the same.

Similar marks of reference denote the same parts.

Roofing material has heretofore been prepared by passing sheets of paper or other material through melted pitch, asphalt, and similar material. Said paper or other fabric is, however, liable to be torn, and the material has to be in a very soft or fluid state, and is often unequally spread upon such fabric. Native asphalt contains from sixty to eighty per cent. of earthy matters, and is the most durable roofing substance of this character known. Artificial asphalt or pitch derived from the distillation of coal-tar, when used alone, is liable to run in hot weather, to crack in cold weather, and rapidly wears away by exposure to the atmosphere. When this artificial asphalt is combined with a large quantity of earthy matters it forms a natural and very durable water-proof cement.

Heretofore roofing fabrics have been coated by passing them through the bituminous composition when in a melted and very fluid condition, and it is impossible to obtain this fluid condition when any considerable amount of earthy matters are mixed in with the composition, because these earthy matters make the compound very thick and stiff. Consequently it has been wholly impracticable in the processes heretofore used to coat felt and similar fabrics with the best kind of composition—that is, one composed of bitumen or similar substance combined with a large amount of earthy matters. This composition of asphalt and earthy matters can be furnished at a much less cost than the simple bitumen or pitch, and I have devised a mode by which it can be applied to roofing fabrics.

The nature of my said invention consists in

a mode of coating roofing fabrics by a pair of rollers in a horizontal position, the space between which forms a hopper for the reception of asphalt or other material, which is applied by the rollers in a uniform layer to a sheet or sheets of felt or other material passed between the coating material and the roller. By this means the coating material is only brought into contact with the sheet of felt or other fabrics, as the sheet itself lies against and is supported by the roller. Hence there is no tendency to tear said sheet, and it does not have to be drawn through the coating material, as heretofore. I am able to add by each pair of rollers a sheet of felt or other material to two or more sheets previously cemented together, so as to produce a roofing fabric of any desired thickness. By this mode of applying the coating material I am enabled to employ it in a much stiffer condition than would be possible if the paper were drawn through it, and I can also introduce with the asphalt or other material earthy matter that will render the roofing material much more durable, but would render the coating material too stiff for use in the manner heretofore practiced.

In the drawings, *a* is a frame of suitable size, receiving the rollers *b b*, *c c*, and *d d*, each pair of which is connected by gears *e e*, and they are all to be propelled by suitable power.

I have represented my apparatus as adapted to the preparation of roofing material from three rolls of paper or other fabric, *f g*, and *h*; but said apparatus may have a greater or less number of pairs of rollers, so as to operate upon a less or greater number of rolls of fabric. The fabric from the rolls *f* and *g* passes under shears or rotary cutters *i*, by which the sheets are brought to a uniform width. Then said fabric passes between the pairs of rollers *b b*. The asphalt or other cement is applied in a semi-fluid state between the rollers *b b*, as represented, and, being soft, adheres to the sheets of paper or other fabric and causes them to stick firmly together as they pass through between the rollers *b b*, the surplus material being squeezed out and kept back. The journal-boxes of one of the rollers *b* should be adjustable, so as to allow for different thicknesses of material, and for varying the thickness of the intervening layer of cement. The other pairs of rollers should also be adjusta-

ble for the same purpose. The two layers of paper or other fabric are led between the rollers *c c*, and at this point the third layer from the roll *b* is added, a rotary cutter being provided at *k* for dressing the sheet to a uniform width, and the asphalt or other cement being applied in a soft state between the layers, when they are pressed together by the rollers.

A surface of asphalt or similar material may be applied to the roofing fabric prepared as aforesaid, by passing the same through the pair of rollers *d d*, at which point the coating material is applied in a soft or semi-fluid state, and is passed or rolled upon the surface of the said roofing material. The roller with which said asphalt comes in contact should be kept greased or so prepared that the asphalt or other material will not adhere thereto.

I do not limit myself to any character of roofing paper, felt, or cloth, but intend to use this apparatus upon any desired character of fabric.

The cutters *i* and *k* might act at the ends of the rollers and form with the edges at this point rotary shears, and the plastic asphalt or other material may be kept in its place by stationary pieces at the ends or between the rollers, to form hoppers for retaining said material.

What I claim, and desire to secure by Letters Patent, is—

The method of coating a sheet or sheets of felt or other material, to form a roofing fabric, with asphalt or other material in a soft or plastic state, applied directly to such fabric in the manner specified.

In witness whereof I have hereunto set my signature this 3d day of February, 1865.

ALFRED ROBINSON.

Witnesses:

THOS. GEO. HAROLD,  
CHAS. H. SMITH.